

# UNITED STATES PATENT OFFICE.

CLAUDE MARIE SANLAVILLE, OF LE COTEAU, FRANCE.

## PROCESS OF MANUFACTURING ARTIFICIAL HORSEHAIR.

1,093,295.

Specification of Letters Patent. Patented Apr. 14, 1914.

No Drawing.

Application filed October 18, 1912. Serial No. 726,492.

*To all whom it may concern:*

Be it known that I, CLAUDE MARIE SANLAVILLE, a citizen of the French Republic, residing at Le Coteau, Loire, in France, 5 have invented a certain new and useful Process of Manufacturing Artificial Horsehair, of which the following is a specification.

The present invention relates to a process 10 of manufacturing artificial or vegetable horsehair intended to replace animal horsehair in its usual applications, and particularly in upholstery, saddlery, strap making, etc.

15 The artificial horsehair is obtained by treating dried alfa sticks or decorticated aloe fiber whereby they are given the suppleness, elasticity, transparency and crispness of animal horsehair. The artificial 20 horsehair has the advantage of being of low cost, does not retain the dust, it possesses resistant qualities, and may be produced in long lengths; further it has an agreeable softness to the touch.

25 The artificial horsehair is prepared by first freeing the lengths of alfa or aloe from the gum which they contain, for example by the following treatment. 100 kilograms of dried alfa sticks or of decorticated aloe 30 fiber are placed with about 1500 liters of water in an autoclave to which 23 liters of caustic soda has been previously added at 36° Baumé, the mixture is then caused to boil for 6 hours while maintaining the pressure at about three atmospheres. After the 35 boiling the pressure is allowed to fall and the bath is emptied and the fibers thoroughly rinsed with water. After the fibers have been freed from gum they are dried 40 and are then ready for the treatment imparting the crispness, suppleness and elasticity of animal horsehair. This treatment

45 consists in immersing the dried fibers in a cold bath of caustic soda at a strength of at least 18° Baumé. The duration of the immersion is about an hour and a half after which the fibers are withdrawn from the bath and again dried. The fibers are finally immersed for a quarter of an hour in an acid bath consisting of 1 liter of sulfuric 50 acid and 100 liters of water whereupon they are thoroughly rinsed to get rid of all trace of acid and are then dried.

55 What I claim as my invention and desire to secure by Letters Patent of the United States is:—

1. A process of manufacturing artificial horsehair from vegetable fibers, consisting in boiling said fibers in a weak solution of caustic soda to free said fibers from gum, 60 then rinsing and drying said fibers, treating them in a cold bath of caustic soda at 18° Baumé or more, again drying the fibers, immersing same in an acid bath to twist and curl the fibers and finally rinsing and drying said fibers.

2. A process of manufacturing artificial horsehair from alfa or aloe fibers consisting in first boiling said fibers at a pressure of about three atmospheres in a weak solution 70 of caustic soda to free said fibers from gum, rinsing and drying the fibers, and immersing them in a cold bath of caustic soda at 18° Baumé or more and again drying said fibers, and finally treating said fibers in a 75 1% sulfuric acid bath and rinsing and drying the same.

In witness whereof I have signed this specification in the presence of two witnesses.

CLAUDE MARIE SANLAVILLE.

Witnesses:

HERBERT FELIX,  
JOSEPH VERNES.